

Feb. 7, 1939.

E. R. BORHO

2,145,858

PROCESS FOR PRODUCING FABRIC AND THE FABRIC

Original Filed Nov. 21, 1933



FIG. 1



FIG. 2



FIG. 3



FIG. 4

INVENTOR

ERNEST R. BORHO

Bohleber & Ledbetter  
ATTORNEYS

## UNITED STATES PATENT OFFICE

2,145,858

PROCESS FOR PRODUCING FABRIC AND  
THE FABRIC

Ernest R. Borho, North Bergen, N. J.

Application November 21, 1933, Serial No. 699,035  
Renewed October 26, 1937

21 Claims. (Cl. 28—1)

The invention relates to a method or process of producing a fabric at least part of which is rendered destructible to produce a fabric having pattern effects therein or to produce a fabric which is entirely destructible. The fabric which is entirely destructible is adapted to be used as a support or a background fabric in the manufacture of embroidery. Partially destructible fabric is suitable for producing a fabric having pattern effects therein or for supporting fabric in the manufacture of embroidery.

The pattern effects produced in a finished patterned fabric are similar to those which are manufactured upon looms in which the yarn of the fabric in certain parts will be closely woven, or relatively closely woven, and other parts will have the effect of being loosely woven such as a net or open work. In producing a fabric having pattern effects, portions of the yarn of the fabric are rendered friable or destructible by the process or method to be described, which friable portions are removed from the fabric and leave the remainder of the yarns intact.

The process of the invention will also produce a fabric, all or part of which will be rendered friable or destructible for use in the manufacture of embroideries. Such fabric is used as a background and supporting fabric and the embroidery is manufactured thereupon, after which the fabric is subjected to treatment which renders it entirely or partially friable or destructible. Thereafter the friable fabric is removed by brushing, crushing, beating, or other suitable manner, which leaves the finished embroidery entirely free of and separated from the background fabric or the embroidery is carried on the supporting fabric which has pattern effects or is net like.

It is an object of the invention to devise a new and novel method of producing a fabric of yarns, at least some or all of which are vegetable or of vegetable origin and at least a portion or all of which vegetable yarns is rendered friable or destructible.

Another object is to devise a new and novel method of producing pattern effects upon fabric having vegetable yarns therein by subjecting the fabric to a treatment which renders some of the yarn or parts of all of the yarn friable or destructible, as desired, whereupon the friable portions are removed leaving the remaining yarn of the fabric to form the pattern effects desired.

Other objects of the invention will be more apparent from the following description taken in connection with the accompanying drawing il-

lustrating one embodiment of the invention in which:

Figure 1 is a plan view of the fabric with the yarns shown partially diagrammatically in order to better illustrate the pattern effect produced by the process. 5

Figure 2 is an enlarged plan view of a part of the fabric showing how the yarn, forming the net or background portion of the fabric, retains the shorter lengths of yarn which form the pattern. 10

Figure 3 is an enlarged cross-section through the background or network of the fabric as taken on line 3—3 of Figure 2.

Figure 4 is an enlarged cross-section through the fabric where a pattern appears in the fabric as taken on line 4—4 of Figure 2. 15

Pattern effects upon fabric having yarns of vegetable fiber or of vegetable origin have been produced heretofore by various processes. One such process nitrates vegetable yarn, after which the fabric or cloth produced from the yarn is printed with a paste containing caustic soda. This process, however, is subject to several disadvantages. 20

Another process impregnates vegetable yarn with a solution of aluminum chloride or magnesium chloride. The treated yarn is woven into cloth which is subsequently printed with an alkali, such as sodium carbonate, in that portion 30 of the fabric where the yarn is to be retained. This treated cloth is then heated which disintegrates the yarns or renders them friable or destructible in those parts not treated with the soda, and the disintegrated portions are removed 35 by brushing, beating, etc.

The above process produces an impregnated yarn and cloth which cannot be stored for any length of time without a loss of yarn, unless great care is taken. The yarns and cloths so treated 40 must also be kept cool and protected from moisture.

Another method utilizes a paste having a free acid therein which is printed upon the fabric in those places where the fabric is to be disintegrated or rendered friable. The paste is permitted to remain upon the fabric until it has disintegrated the same, after which the paste is washed therefrom. This method has the disadvantage of the acid attacking the equipment 50 for producing the pattern effects.

The process for producing a fabric to be described herein is adapted to be performed upon vegetable fibers or fibers having a vegetable origin. The fabric need not necessarily be en- 55

tirely of yarns from vegetable fibers although, in the preferred fabric, it is contemplated to weave or manufacture the fabric entirely of vegetable fibers because of the greater desirability of this fiber and yarn in most cases. Cotton is the cheapest of the vegetable fibers and consequently yarns of cotton or cotton origin will probably be most frequently used in practicing the process. Any yarn, however, of vegetable fiber or vegetable origin is suitable for practicing the process and for the purposes of this invention the term vegetable yarn includes all such yarns.

The vegetable yarns which are to be treated are first thoroughly scoured in the recognized manner for the particular yarns used. This is merely a conditioning treatment which all yarns receive before further processing and does not constitute one of the steps in the process of the invention. The first operation in the inventive process comprises the treating of the vegetable yarns 10 with a compound containing one or more diazotizable amino groups which are absorbed into the fibers of the yarn and retained therein. It is important that the diazotizable amino group compound be absorbed and retained in the fiber initially and after diazotization and one of the factors determining the relative practicability of one diazotizable amino group compound over another in performing my process is the quantity of compound absorbed and retained by the fiber. Other factors being the same, the relative substantivity or ability of the fiber to absorb and retain more of one diazotizable amino group compound than another makes the one which is more substantive more satisfactory.

The vegetable fibers are treated with the diazotizable amino group compound either as an aggregate of fiber or as yarn before it is manufactured into a cloth or fabric, or the yarns or fiber may be treated after the yarns have been woven into the fabric, although for producing pattern effects the treatment of the fiber before spinning into yarn or before weaving the yarn into fabric is preferable as will appear more fully herein-after. Pattern effects may be produced by treating portions of yarns with the diazotizable amino group compound and weaving these yarns 10 into fabric and then disintegrating the treated portions. Obviously, such yarns may also be woven into fabric with yarns 11 which are untreated, or with yarns which have been entirely treated, or with both of these forms of yarn.

A fabric having more intricate pattern effects may be produced by taking one of the fabrics, above described, or a fabric in which all parts of all the yarns are treated with a diazotizable amino group compound and applying thereto a compound or chemical which reduces or oxidizes the diazotizable amino group compound so that it is in a condition to be removed from the yarns of the fabric or changes its character or composition so that it no longer contains an effective diazotizable amino group. Such reducing agents as sodium hydrosulphite, stannous chloride and titanous chloride are well known and commonly used reducing agents in the textile industry, and sodium chlorate is an oxidizing agent which has the same effect of removing the diazotizable amino group compound from the fabric in those portions where it has been applied for the purpose of retaining the yarns. Of these reducing and oxidizing agents, sodium hydrosulphite is preferred in my process.

The preferred manner of applying this reducing or oxidizing agent to the fabric is by printing

a paste thereof in a desired pattern on the fabric in those places where the treated yarns 10 are to be retained. The primary purpose of this step is to have the diazotizable amino group compound absorbed in the treated yarns in the fabric only where desired in a predetermined pattern. The fabric is now dried, steamed and washed to remove the paste containing the oxidizing or reducing agent and to remove any residual substances from the fabric. It will be noted that the purpose of the removing or discharging step in the process is to remove the diazotizable amino group compound or so change the character thereof that it is rendered ineffective.

The diazotizable amino group compound in the fabric is diazotized. The preferred manner of diazotizing the compound is to subject the fabric to a cold diazotizing bath of any soluble nitrite, such as sodium nitrite or potassium nitrite, and a mineral acid, such as sulphuric acid, hydrochloric acid, ortho-phosphoric acid or nitric acid. The sulphuric and hydrochloric acids are preferred since these acids have been found more effective than the other acids. It is essential that the diazotization of the amino group compound will produce a diazonium salt which is retained in the fiber of the fabric. The fabric after being treated to the diazotizing step, is thoroughly washed with cold water to remove all acid and nitrite.

Some of the yarns of the fabric resulting from the steps of the process so far described contain a diazonium salt in a desired pattern and the remainder of the yarns of the fabric do not contain the diazonium salt. The diazonium salt is unstable and will decompose at normal temperatures and under normal atmospheric conditions and produces an active disintegrating agent. Because of this fact, the fabric is immediately dried after removal from the diazotizing bath in order to avoid the disintegrating agent from spreading outside of the pattern limits as might occur if the fabric were in a moist condition. The liberation and activity of the disintegrating agent proceeds relatively slowly at ordinary temperatures.

In order to increase the speed with which the disintegrating agent is liberated, the fabric is heated to a temperature and for a period of time which will not be injurious to the retained yarns. The diazonium salt when so heated rapidly liberates the active agent which disintegrates or renders the yarn friable in those places containing the diazonium salt, which are those places where the diazotizable amino group compound has been impregnated into the yarn or has been permitted to remain in the yarn of the fabric. The temperature, to which the fabric may be subjected, is governed by other conditions such as the length of time to which the fabric is subjected thereto, and the dehydration within the yarns which must necessarily take place under the temperature applied. The heating of the fabric must avoid carrying the dehydration to the point where the yarns retained are injured. The fabric may be subjected to very high temperatures for a short period, provided the yarns which are to be retained in the fabric are not scorched or otherwise injured by the heat.

The friable or disintegrable yarn produced in the fabric is reduced to a powder or minute broken pieces by pounding or crushing, brushing, or by any other suitable method. This leaves a fabric with pattern effects in which the yarns 10 and 11 of the fabric in certain portions thereof are closely or relatively closely woven and in

other portions some or all of the yarns have been removed producing a net or open-work effect. If the fabric is one having a pile and the process has been applied to the yarns of the pile, a pattern effect in the pile would be produced. Similarly, the process is applicable to the yarns in the ground of a pile fabric which would also produce pattern effects therein. Combinations of patterns in the pile and in the ground may be obtained, as desired. The fabric is now ready for any other of the usual treatments to which a fabric may be subjected, such as singeing, scouring, bleaching, mercerizing, dyeing and finishing.

The process of producing a fabric, described above, may also be used to produce background and supporting fabric in the manufacture of embroidery. Embroidery is often manufactured upon a fabric, all of which fabric is subsequently destroyed leaving the embroidery without any of the background fabric remaining. Again the supporting fabric may be partially retained as a supporting net or open-work fabric for the embroidery or may have any desired pattern therein. In producing fabric for the embroidery manufacturing trade, the same steps are performed as outlined above, excepting in a fabric all of which is to be destroyed in which case the step of removing the diazotizable amino group compound is dispensed with.

For a fabric which is to be entirely destroyed, all of the yarns are impregnated with the diazotizable amino group compound, either as yarns which are then woven into the fabric, or the yarns may be treated after being woven into a fabric. In removing the diazotizable amino group compound from certain portions of the fabric, this step is taken in order to produce desired pattern or open-work effects in the fabric. Obviously, where no pattern effects are desired and all that is wanted is the entire destruction of the fabric, this step should not be performed. Again, such a fabric must have all of the yarns woven into the fabric treated in the manner described so that the entire fabric becomes friable or destructible upon heating.

The fabric produced by the invention is much superior to any now being used by the embroidery manufacturing trade. The fabrics now used cannot be stored since the disintegration or conversion of the vegetable yarn into a friable condition proceeds immediately in spite of all precautions taken to protect the same against actinity. Furthermore, one of the fabrics now used is highly inflammable. The fabric produced by the method disclosed herein may be stored indefinitely until ready for use without deterioration and the fabric may be rendered friable after the embroidery has been manufactured thereupon merely by diazotizing the fabric and subjecting it to heat, as described above. The fabric produced by the process described herein is also no more inflammable than any vegetable yarn fabric.

Another advantage of the fabric produced by the method described is that it has definite color. The majority of embroideries are manufactured with a light colored yarn. The background or supporting fabric heretofore used in the embroidery manufacturing industry is inherently a light colored fabric and consequently the light colored embroidery yarn does not show up effectively. For this reason these fabrics have been dyed as a separate and additional step in the manufacture of the fabric. The compound

which is most effective for the process described herein produces a fabric which is initially black without requiring a separate dyeing step. Other diazotizable amino group compounds which can successfully be used produce a distinct or deep color in the fabric without an additional dyeing step. These distinct colors of the fabric provide a sharply contrasting background for the light colored yarns of the embroidery so that the embroidery pattern is readily discernible upon the background fabric.

The diazotizable amino group compounds which are suitable for the process described herein must be substantive or absorbed and retained in sufficient quantities in the fibers of the yarn. Those diazotizable amino group compounds which are most successful have been found to be those having a maximum number of diazotizable amino groups therein and which have also maximum substantivity. It has been found, for instance, that some of the diazotizable amino group compounds having two diazotizable amino groups are not as effective for the process as some compounds having only one diazotizable amino group. It is believed that one of the reasons why the compound containing the single diazotizable amino group is more effective than the compound containing the two diazotizable amino groups is because of the relative substantivity of the two compounds, the former being probably absorbed and retained in the fibers of the yarn in much larger quantity than the latter. In other words, a compound having two diazotizable amino groups therein is not absorbed and retained in the fiber of the yarn in a quantity sufficient to provide the same number of diazotizable amino group units therein as the units absorbed and retained in the fiber in a compound containing a single diazotizable amino group yet being relatively more substantive. Again the diazotization of the substantive diazotizable amino group compound has for its purpose the production and retention of a diazonium salt in the fibers of the yarns in sufficient quantity to provide an adequate amount of active disintegrating agent within the fiber.

In the preferred method described herein of producing a fabric having pattern effects, wherein the diazotizable amino group compound is reduced or oxidized from desired portions of the fabric, it is essential that a diazotizable amino group compound be used which is removable or rendered ineffective to produce the active disintegrating agent. In practicing the preferred method of producing pattern effects, therefore, a diazotizable amino group compound must be used which is substantive and capable of being removed preferably in a printing process such as is now practiced in the textile industry. Some diazotizable amino group compounds which have been particularly effective for embroidery supporting fabrics and for producing pattern effects by the preferred method are:

Sodium salt of 4 amino-benzene-azo-*p*-creasol-methyl ether-azo-7 amino-1 naphthol-3 sulphonic acid.

Sodium salt of diphenyl-disazo-3-sulpho-7 amino-1 naphthol-3:6 disulphonic acid.

Sodium salt of *p* aminobenzene-azo- $\alpha$  naphthene-azo-7 amino-1 naphthol-3 sulphonic acid.

Sodium salt of *m*-aminobenzoyl-6 amino-3 sulpho-1 naphthol-2 azo-benzene.

The first mentioned has so far been found most effective.

Various modifications will occur to those skilled

in the art in the steps going to make up the invention as a whole, as well as in the selective combination or application of the respective steps, and no limitation is intended by the phraseology of the foregoing description.

What is claimed is:

1. A process for producing a fabric at least some of which is of vegetable yarns and at least some of which vegetable yarns have a diazotizable amino group compound absorbed and retainable therein comprising, diazotizing the diazotizable amino group compound, then drying the fabric so that the yarns thereof to be removed are rendered friable and the remaining yarns are uninjured, and removing the friable portions of the fabric. 5
2. A process for producing a fabric at least some of which is of vegetable yarns and at least some of which vegetable yarns have a diazotizable amino group compound absorbed and retainable therein comprising, diazotizing the diazotizable amino group compound, then heating the fabric to dry the yarn and so that the yarns thereof to be removed are rendered friable more quickly and the remaining yarns are uninjured, and removing the friable portions of the fabric. 10
3. A process for producing a fabric at least some of which is of vegetable yarns and at least some of which vegetable yarns have a diazotizable amino group compound absorbed therein comprising, diazotizing the diazotizable amino group compound, drying the fabric, then heating the fabric so that the yarns thereof to be removed are rendered friable quickly and the remaining yarns are uninjured, and removing the friable portions of the fabric. 15
4. A process for producing fabric at least some of which is a vegetable yarn comprising, treating yarn which is to be removed with a compound having a diazotizable amino group which is absorbed and retained in the fiber of the yarn, diazotizing the diazotizable amino group compound, then drying the fabric so that the yarns or parts thereof to be removed are rendered friable and the remaining yarns are uninjured, and removing the friable yarns of the fabric. 20
5. A process for producing fabric at least some of which is a vegetable yarn comprising, treating yarn with a compound having a diazotizable amino group which is absorbed and retained in the fiber of the yarn, removing the diazotizable amino group compound from so much of the yarn which is to be retained, diazotizing the diazotizable amino group compound, then heating the fabric so that the yarns or parts thereof to be removed are rendered friable and the remaining yarns are uninjured, and removing the friable yarns of the fabric. 25
6. A process for producing patterned fabric at least some of which is a vegetable yarn comprising, treating yarn with a compound having a diazotizable amino group which is absorbed and retained in the fiber of the yarn, applying a compound upon so much of the yarns of the fabric which are to be retained which removes or renders ineffective the diazotizable amino group compound, washing the fabric, diazotizing the diazotizable amino group compound, then heating the fabric so that the yarns thereof to be removed are rendered friable and the remaining yarns are uninjured, and removing the friable yarns of the fabric. 30
7. A process for producing fabric comprising, treating a vegetable yarn prior to weaving with a compound having a diazotizable amino group which is absorbed and retained in the fiber of the 35
- yarn, weaving the yarn into a fabric, diazotizing the diazotizable amino group compound, washing the fabric to remove all acid and nitrite, heating the fabric, and removing the friable yarns. 40
8. A process for producing fabric comprising, weaving a fabric of yarns at least some of which are vegetable, treating the fabric with a compound having a diazotizable amino group which is absorbed and retained in the fiber of the yarn, diazotizing the diazotizable amino group compound in the yarn, and drying the fabric. 45
9. A process for producing fabric comprising, treating a vegetable yarn prior to weaving with a compound having a diazotizable amino group which is absorbed and retained in the fiber of the 50
- yarn, weaving the treated yarn into a fabric with other untreated threads, diazotizing the diazotizable amino group compound, then drying the fabric so that the portions of the yarns thereof to be removed are rendered friable and the remaining yarns and portions thereof are uninjured, and removing the friable portions of the 55
- yarns of the fabric. 60
10. A process for producing fabric comprising, treating a vegetable yarn prior to weaving with a compound having a diazotizable amino group which is absorbed and retained in the fiber of the yarn, weaving the yarn into a fabric with other untreated threads, removing the diazotizable amino group compound where desired, diazotizing the remaining diazotizable amino group compound, then heating the fabric so that the yarns thereof to be removed are rendered friable and the remaining yarns are uninjured, and removing the friable portions of the 65
- fabric. 70
11. A process for producing a fabric at least some of which is of vegetable yarns and at least some of which vegetable yarns have a diazotizable amino group compound absorbed and retainable therein comprising, diazotizing the diazotizable amino group compound, then drying the fabric at normal temperatures so that the fabric is dry for storage and the disintegrating agent is unliberated. 75
12. A process for producing patterned fabric at least some of which is a vegetable yarn comprising, treating yarn with a compound having a diazotizable amino group which is absorbed and retained in the fiber of the yarn, weaving the treated yarn into a fabric with other yarns, applying hydrosulphite upon so much of the yarns of the fabric which are to be retained which removes or renders ineffective the diazotizable amino group compound, washing the fabric, diazotizing the diazotizable amino group compound, then heating the fabric so that the yarns thereof to be removed are rendered friable and the remaining yarns are uninjured, and removing the 80
- friable yarns of the fabric. 85
13. A process for producing patterned fabric at least some of which is a vegetable yarn comprising, treating yarn with at least one of the compounds of sodium salt of 4 amino-benzene-azo-creasol-methyl ether-azo-7 amino-1 naphthol-3 sulphonic acid, sodium salt of diphenyl-disazo-3 sulpho-7 amino-1 naphthol-3:6 disulphonic acid, sodium salt of *p*aminobenzene-azo-anaphthalene-azo-7 amino-1 naphthol-3 sulphonic acid, sodium salt of *m*-aminobenzoyl-6 amino-3 sulpho-1 naphthol-2 azo-benzene which is absorbed and retained in the fiber of the yarn, weaving the treated yarn into a fabric with other yarns, applying hydro-sulphite upon so much of the yarns of the fabric which are to be retained which removes or renders ineffective the diazotizable amino 90
- 95

group compound, washing the fabric, diazotizing the diazotizable amino group compound, then heating the fabric so that the yarns thereof to be removed are rendered friable and the remaining 5 yarns are uninjured, and removing the friable yarns of the fabric.

14. A process for producing patterned fabric at least some of which is a vegetable yarn comprising treating yarn with at least one of the compounds of sodium salt of 4 amino-benzene-azo-*p*-creasol-methyl ether-azo-7 amino-1 naphthol-3 sulphonic acid, sodium salt of diphenyl-disazo-3 sulpho-7 amino-1 naphthol-3:6 disulphonic acid, sodium salt of *p*aminobenzene-azo-*o*-naphthalene-15 azo-7 amino-1 naphthol-3 sulphonic acid, sodium salt of *m*-aminobenzoyl-6 amino-3 sulpho-1 naphthol-2 azo-benzene which is absorbed and retained in the fiber of the yarn, weaving the treated 20 yarn into a fabric with other yarn, applying a compound upon so much of the yarns of the fabric which are to be retained which removes or renders ineffective the diazotizable amino group compound, washing the fabric, diazotizing the diazotizable amino group compound, then heating 25 the fabric so that the yarns thereof to be removed are rendered friable and the remaining yarns are uninjured, and removing the friable yarns of the fabric.

15. In a process for producing patterned fabric at least some of which is a vegetable yarn including the use of one of the diazotizable amino group compounds of sodium salt of 4 amino-benzene-azo-*p*-creasol-methyl ether-azo-7 amino-1 naphthol-3 sulphonic acid, sodium salt of diphenyl-disazo-3 sulpho-7 amino-1 naphthol-3:6 disulphonic acid, sodium salt of *p*aminobenzene-azo-*o*-naphthalene-azo-7 amino-1 naphthol-3 sulphonic acid, sodium salt of *m*-aminobenzoyl-6 amino-3 sulpho-1 naphthol-2 azo-benzene, and 40 including the use of a compound upon so much of the yarns of the fabric which are to be retained which removes or renders ineffective the diazotizable amino group compound.

16. In a process for producing patterned fabric at least some of which is a vegetable yarn including the use of a compound having a diazotizable amino group which is absorbed and retained in the fiber of some of the yarn of the fabric, and including the use of a compound upon so much of the 45 yarns of the fabric which are to be retained which removes or renders ineffective the diazotizable amino group compound.

17. A fabric having a pattern effect, in which twisted threads extend entirely across the fabric, other shorter threads retained therebetween by the twisted threads and forming a desired pattern, and the shorter threads being initially long threads dyed with a dye having a diazotizable 50

amino group which is retained on the fiber after which the dye is removed therefrom where the shorter thread is desired so that it remains to form the pattern and the balance of the thread is removed.

18. A process for destroying all or a portion of a fabric at least some of which is of vegetable yarns and at least some of which vegetable yarns have a diazotizable amino group compound which is absorbed and retained therein and its diazonium salt is also retained therein comprising diazotizing the diazotizable amino group compound within and upon the fibers of the yarns thereby forming the diazonium salt, then drying the fabric so that the yarns thereof to be removed are 15 rendered friable and any remaining yarns are uninjured, and removing the friable portions of the fabric.

19. A process for destroying all or a portion of a fabric at least some of which is of vegetable 20 yarns and at least some of which vegetable yarns have a diazotizable amino group compound which is absorbed and retained therein and its diazonium salt is also retained therein comprising, diazotizing the diazotizable amino group compound within and upon the fibers of the yarns thereby forming the diazonium salt, then heating the fabric to dry the yarn and so that the yarns thereof to be removed are rendered friable more 25 quickly and any remaining yarns are uninjured, and removing the friable portions of the fabric.

20. A process for destroying all or a portion of a fabric at least some of which is of vegetable yarns and at least some of which vegetable yarns have a diazotizable amino group compound which is absorbed and retained therein and its diazonium salt is also retained therein comprising, diazotizing the diazotizable amino group compound within and upon the fibers of the yarns thereby forming the diazonium salt, drying the fabric, 40 then heating the fabric so that the yarns thereof to be removed are rendered friable quickly and any remaining yarns are uninjured, and removing the friable portions of the fabric.

21. A process for destroying all or a portion of a fabric at least some of which is a vegetable yarn comprising, treating yarn which is to be removed with a compound having a diazotizable amino group which is absorbed and retained in the fiber of the yarn and its diazonium salt is also retained 45 therein, diazotizing the diazotizable amino group compound within and upon the fibers of the yarn thereby forming the diazonium salt, then drying the fabric so that the yarns or parts thereof to be removed are rendered friable and any remaining yarns are uninjured, and removing the friable 50 yarns of the fabric.

ERNEST R. BORHO.